



high current density so long as the acid is maintained at a fairly strong concentration.

In order to appreciate the invention, I shall in the following describe in detail the several parts of my apparatus and the various steps of the method.

In parting and refining, according to my invention, I may start with a wide variety of commercial and other forms of impure gold as the anode. Jewelry gold, for example, ten carat to eighteen carat (.417 to .750 fine) grades, and the scrap bullion offered for refining, generally .400 to .600 fine may be refined with my process. Platinum and palladium are invariably present in this scrap bullion in amounts varying from a trace to as high as two percent which indicates the admixture of dental scrap. Lead also is generally present in this nondescript alloy. Dental gold usually has a high gold content and may contain up to twenty-five percent platinum and palladium. The dental scrap bullion averages about 18 carat. In recent years, alloys containing 25 to 50% palladium have come into use with correspondingly lower percentages of gold and platinum.

High grade scrap bullion which may be refined by my process is generally a mixture of jewelry and dental scrap, a typical composition being:

|                                                                                                | Per cent |
|------------------------------------------------------------------------------------------------|----------|
| 30 Gold                                                                                        | 60       |
| Silver                                                                                         | 15       |
| Copper                                                                                         | 17       |
| Zinc                                                                                           | 4        |
| 35 Nickel                                                                                      | 1        |
| Balance consisting of tin, lead, iron, platinum, palladium, other metals, silicon and sulphur. |          |

Low grade scrap bullion which I may also treat, consists mainly of rolled - gold - plate scrap. Rolled-gold-plate or gold-filled is a shell of gold from 10 k. to 14 k. soldered with silver solder to a base metal. The gold may be on one or both sides or may be a seamless shell on wire. A typical composition of scrap bullion of this class would be:

|                                                                             | Per cent |
|-----------------------------------------------------------------------------|----------|
| Gold                                                                        | 4.0      |
| Silver                                                                      | 1.5      |
| 50 Copper                                                                   | 70.0     |
| Nickel                                                                      | 4.0      |
| Zinc                                                                        | 17.0     |
| Tin                                                                         | 2.0      |
| Balance lead, iron, platinum, palladium, other metals, silicon and sulphur. |          |

The base bullion anodes may be cast in an open mold with a small head or lug at the top and a one-eighth inch diameter copper or silver wire inserted in the lug before the metal solidifies. The conducting wire may be welded to the lug with a torch flame, if desired. The upper end of the anode is cast thicker than the lower to compensate for localized high current densities.

The cathodes may consist of strips of sterling silver, fine gold or tantalum, or preferably sterling silver plated or faced with the fine gold or a metal of the platinum group. Sterling silver tubing may serve as cathodes and cooling water may be passed through them to cool the bath. They may be bolted or soldered to the cathode conductor bars which may be made, preferably, of copper electro-plated with silver or gold. The anode conductor wire may be bolted to the anode cross bar

with a small brass bolt. Well known means for agitating the electrolyte are provided.

The electrolyte is concentrated (commercial grade) hydrochloric acid. In this case, if anodes .600 fine with 15% silver and 25% copper are used, a current density of about 300 amperes per square foot of anode surface may be employed. At 180 amperes per square foot, an anode-efficiency of about 63% is realized with anodes of this composition. By adding even a slight amount of sodium chloride to the electrolyte with the same anodes, the current density may be increased to 630 amperes per square foot or more without generating chlorine at the anode. Using a current density of 180 amperes, the anode efficiency increased to 75% as compared to the efficiency without sodium chloride of 63%. I have noticed similar effects in using potassium, calcium and barium chlorides.

No external heat is applied, the bath being self-heating. Some cooling is required to prevent boiling, but I prefer to provide sufficient cooling to maintain the bath temperature below 35° C.

The electrochemical effects visible during electrolysis are as follows: Let us assume that we start with an anode of a composition within the usual range—say, about 60% gold, 15% silver, and 15 to 25% copper. At the beginning of electrolysis, with fresh concentrated hydrochloric acid, the anode goes into solution in the electrolyte and if the bath is not agitated, the dark green solution sinks to the bottom of the cell so that little or no deposit is formed. Silver chloride is formed at the anode, most of it dropping off immediately or adhering loosely, and a small amount being dissolved. During this initial period, an assay of the colored liquid would show the presence of gold. There is also strong gassing at the electrodes, oxygen at the anode, and hydrogen at the cathode. This gassing is reduced in amount, and with it the potential across the cell, if salt is added, or if superimposed alternating current is used. As electrolysis continues, the heavy colored solution at the bottom increases in amount and also diffuses to some extent towards the top, especially with rising temperature. As this solution containing the anode metal rises and comes into contact with the cathode, a deposit of gold rapidly forms on the cathode. In addition, a reaction is momentarily noticeable which is always seen during the entire operation of the Wohlwill process, namely, a precipitation of finely divided gold throughout the bath. I assume that this precipitation is the well known decomposition of aurous chloride or chloraurous acid into metallic gold and auric chloride or chlorauric acid. This reaction, however, is only momentary and is not again visible during the continuance of electrolysis. If the bath is stirred or agitated from the beginning, this reaction apparently does not occur. It appears reasonable to assume from the above that aurous ions are not formed at the anode, and that they are formed at the cathode momentarily, when the solution coming into contact with the cathode, contains an excess of auric ions beyond the amount which can be immediately reduced to metallic gold. Almost immediately after deposition begins, the bath becomes depleted of gold and continues in this condition thereafter. Both cupric and cuprous chloride are found in the solution as well as chlorides of the other metals present. The cathode deposit is spongy and continues to drop off the cathode to the bottom of the tank. The cathode deposit usually con-

tains only gold and silver, but if any large amount of platinum group metals is dissolved from the anode, small amounts of these may be present in the cathode deposit.

5 If the gold content of the anode is low and the copper content correspondingly high, the cathode deposit may consist largely of copper mixed with gold and silver.

If the gold content of the anode, however, is 10 high, and no copper is present, as is the case in the electrolytic refining process to be described later, the presence of aurous chloride, as evidenced by the precipitation of finely divided gold, is not apparent at any time during electrolysis.

15 In this case, a certain amount of gold remains in the solution undeposited on the cathode.

The free acid in the bath is gradually consumed in the formation of chlorides of silver, copper, platinum, etc. The anode efficiency and the production rate drop off correspondingly. In one instance, using direct current alone, at an anode current density of 175 amperes per square foot, the average anode loss in weight per 100 ampere hours was 5.15 ounces during the first eight 20 hours of operation. The average for the second eight hours period was 3.50 ounces per 100 ampere hours, the average for the sixteen hours being 4.3 ounces. Thus, at the end of sixteen hours, the bath no longer gives good production. The 25 bath acts somewhat differently when using superimposed alternating current on the direct current, initial anode consumption as high as 7.5 ounces per 100 ampere hours being obtained at the same current density.

30 To improve the average anode efficiency over a longer period of time, the bath may be continuously changed or be removed at intervals such as four or eight hours and also the copper and silver and platinum group metals may be 35 regularly electrodeposited at low current density with insoluble anodes. The acid of the bath is thus renewed to some extent permitting the further use of the bath until impurities accumulate in sufficient amount to interfere with the gold 40 cathode deposit. As the action proceeds, the electrolyte contains a relatively high amount of silver chloride in solution which does not precipitate on cooling but precipitates on dilution of the bath with water. Cuprous chloride and iron 45 silicate similarly precipitate.

The electrolytic action is accompanied by strong polarization and evolution of oxygen at the anode and hydrogen at the cathode. The polarization and gassing is reduced by addition of 50 a soluble chloride and by use of superimposed alternating current or rectified alternating current. The voltage under these conditions must always exceed 1.7 volts.

The actual voltage applied depends on anode 55 composition, current density desired, electrode spacing, agitation of bath, temperature, composition of electrolyte and several other conditions. Under average conditions, a cell potential of 4 to 4.5 volts is sufficient for a current density of 60 600 amperes per square foot.

The resulting cathode deposit is a loose spongy mass of gold filled with hydrogen gas. It builds up thickly on the cathode and soon drops off by its own weight to the bottom of the tank, where 65 it mixes with silver chloride and anode particles which have also dropped down. The tank slimes are removed at convenient intervals, filtered, washed with hot water and refined by any suitable method, to obtain fine gold. An assay of 70 the metallic part of the slimes (after removing 75

the admixed AgCl by leaching with a solvent) shows gold .920 to .986 fine, if anodes of the usual range of composition are used. The balance is mainly metallic silver, only traces of other metals being found as a rule.

If the amount of gold in the anode is low, other metals such as copper or platinum may be found in greater or less amount in the cathode deposit, but do not hinder the subsequent refining. Under certain conditions, as when much platinum 10 is present in the anode, chlorine may be generated at the anode but the anode continues to pass into solution, nevertheless.

My process thus permits the rapid solution of base bullion anodes at high current density, 15 without regard to the silver content and with practically no interference or retardation from the formation of silver chloride. It also provides for the deposition of fairly pure gold at the cathode in a form that is easily removed and rapidly 20 refined. The success of my method with high silver anodes at high current density, I assume to be at least in part due to the fact that silver chloride partly dissolves under the conditions of 25 my process. I assume it is this extra solubility which prevents the silver forming a passive coating on the anode. The high current density I find it possible to employ is in part due to the fact that AgCl does not interfere with the dissolution of the anode. However, the principal 30 factor permitting the use of high current density is that in my electrolyte, which contains the maximum possible amount of free HCl and other chlorine compounds such as soluble chlorides, gold 35 does not become passive when polarized at the anode at tremendously high current densities. The same is true of palladium and to a lesser degree of platinum.

The solubility of AgCl in hydrochloric acid 40 decreases rapidly on dilution of the acid, but increases rapidly with rising temperature. The solubility of AgCl in acid diluted to 63.5% by volume (20% anhydrous HCl) when heated to 107° C. (boiling point 108.5° C.) approaches its solubility in boiling concentrated acid. The 45 presence of soluble chlorides increases the solubility of AgCl in hydrochloric acid and this effect also increases rapidly with increasing temperature. Although the acid strength diminishes in the course of electrolysis the relatively high 50 solubility of silver chloride is maintained by the increasing concentration of the soluble chlorides of metals dissolved from the anode.

The comparatively large solubility of AgCl in the electrolyte is shown qualitatively by the following: if the bath be slightly diluted with water, a copious precipitate of cuprous chloride and silver chloride is formed which redissolves on boiling. If a large amount of water be added, the AgCl precipitate does not redissolve on boiling, to 55 any visible amount.

This solubility of AgCl leads to one slight difficulty. That is, the deposition of metallic silver at the cathode to the extent of 1.5% to 8% of the total cathode deposit, being apparently 60 alloyed with the gold. This silver content somewhat retards, but does not seriously interfere with the refining of the cathode deposit, when refined by the aqua regia or the Wohlwill methods. This silver content can be controlled to a 65 large degree by the use of high cathode current density, by cooling, and by using superimposed alternating current or rectified current, or with an auxiliary electrolysis to remove the silver from the electrolyte before the latter comes into con- 70 75

tact with the cathode. With superimposed alternating current and a cathode density about 350 amperes per square foot, I have been able to reduce the cathode silver to 1.4%. In the same 5 test, cathode density of 180 amperes per square foot gave a silver content of 3.72% with superimposed alternating current and with direct current alone, 6.22%.

Lead in the anode acts similarly to silver, but 10 lead chloride is more soluble than silver chloride in a hot bath. For this reason, sulphuric acid is added to the Wohlwill bath, to form lead sulphate, which is practically insoluble. Lead sulphate forms a passive coating similar to silver chloride, but as the amount of lead is usually small, it does not interfere. I have found that in the Wohlwill bath containing more than the usual amount of gold and of hydrochloric acid, the addition of sulphuric acid was not effective 15 20 if the anode contained much lead, the bath being filled with lead chloride crystals when cold. In my present process although lead is always present in the anode, I have at no time encountered trouble from this source. The lead is apparently completely dissolved and does not crystallize when cold, and does not usually contaminate the cathode deposit.

The remarkable increase in rate of decomposition of the anode, accompanied by increased 30 anode efficiency, on the addition of sodium chloride, was pointed out hereinabove. Even a minute amount of salt, for example, a pinch of salt in a two gallon cell produces this effect. This effect is still more remarkable, considering the 35 very slight solubility of salt in concentrated hydrochloric acid, about 0.1%.

There would seem to be a relation between the effect of the minute amount of salt and the minute gold content of the bath.

40 If a sample of the bath be taken shortly after electrolysis has started, with ordinary anodes, containing 50-60% gold with the bath agitated, an ordinary qualitative test for gold in solution will be negative. This condition is theoretically 45 impossible, since gold is continuously dissolving from the anode, and a more delicate test would no doubt reveal traces in solution, if a sample be taken near the anode. (With anodes of higher gold content, and a low base metal content, there 50 is, of course, a large proportion of dissolved gold remaining undeposited.) This indicates that copper and other base metals dissolving, displace gold from the bath with extraordinary rapidity. We can consider, for practical purposes, that the 55 gold is deposited as fast as it dissolves, and that traces of salt are sufficient to combine with the traces of gold chloride present, forming a double chloride, which has a lower decomposition voltage than chlorauric acid, and the maximum current 60 density limit of passivity of gold is raised. There may also be an effect of the added chlorine ions on the base metals present.

Fine gold itself exhibits passivity—that is, 65 above a certain current density gold ceases to dissolve and chlorine is set free. This is ascribed by Allmand and Puri (Trans. Faraday Soc. 1925) and others to the formation of an oxide film. Wohlwill found that sodium chloride or HCl 70 added to his chlorauric acid bath formed a double chloride and enabled him to increase the current density. Superimposed alternating current has been found by Allmand and Puri to raise this limiting current density for fine gold 75 anodes in dilute hydrochloric acid, and they also

observed that it was raised by higher temperature as well as by higher acid concentration.

In the Wohlwill process, the limiting factor is the passivating coating of silver chloride. Superimposed alternating current loosens the silver 5 chloride and incidentally raises the gold passivity limit of current density. Hydrochloric acid or sodium chloride has the same effect with respect to gold. The gold effect here is of minor importance, as the silver effect limits the process. 10

My observations have led me to think that the silver content has little or no limiting effect in my process. I have succeeded in decomposing even fine silver rapidly. I believe the only limiting effect present is anode passivity of gold; probably also of platinum, iridium and osmium when present. The presence of salt, forming double chloride, raises the limited current density of gold, and use of superimposed alternating current further raises it. 15 20

The action of anodes with a very high gold content and little or no base metal is shown by the following:

In experiments to use my parting method also as a refining method, I used an anode containing 25 93% gold and 7% silver derived from the cathode slimes as follows: I washed the cathode deposit with ammonia water to remove silver chloride, melted the residue into an anode, and treated the anode by the process in the same manner 30 as for parting as hereinbefore set forth, but the bath was not stirred. Most of the gold dissolved and remained in the bath, while some of it deposited on the cathode in the usual way. When most of the anode had been used up, I added a 35 little nitric acid to the bath and the cathode deposit immediately dissolved, indicating that little or no metallic silver had deposited. After diluting the solution and filtering off the silver chloride, the gold was precipitated and proved to 40 be of high purity.

In another case, I treated anodes of a somewhat unusual composition, approximately:

|           | Per, cent |
|-----------|-----------|
| Platinum  | 8 45      |
| Palladium | 19        |
| Gold      | 15        |
| Silver    | 45        |
| Copper    | 13        |

This worked very satisfactorily in the usual manner. There was no appreciable amount of gold in the bath at the end of the operation, and there was very little platinum metal in the cathode deposit. 50

As stated hereinabove, fine silver can be decomposed rapidly. Pure platinum as anode is attacked less rapidly (with direct current) but nevertheless does dissolve, with liberation of chlorine. 55

If refining the cathode slimes obtained by the above parting process is to be done by the Wohlwill process, the greater part of the silver chloride is preferably removed before melting the anodes. This may be done chemically in for example one of three ways:

- By dissolving and washing with ammonia water.
- By dissolving and washing with sodium thiosulphate.
- By reducing with zinc or copper to metallic silver, which is then removed in hot nitric acid.

Another method is to separate the silver chloride in the course of melting, under oxidizing condi- 75

the gold slimes are about foot square and is recommended to melt a microscopic quantity.

Under such conditions, the silver chloride melting at a low temperature and floating to the top of the metal. This causes some loss of silver by volatilization.

If the slimes are to be refined by acid treatment, the silver chloride need not be removed.

The washed slimes are treated with hot aqua regia until all the gold is dissolved. The solution is evaporated almost to dryness, with additions of hydrochloric acid until all the nitric acid has been driven off.

The crystallized residue or syrupy liquid is dissolved in 5% hydrochloric acid, allowed to stand until all the dissolved silver chloride precipitates and settles, and the solution is filtered.

A reducing agent, such as ferrous sulphate or sodium bisulphite, is added to the filtrate and the gold is precipitated. The precipitate is washed with hot water, dried and melted, and poured into bars, about .9996 fine.

If a higher purity be desired, the gold precipitate is at once redissolved, and reprecipitated.

I propose as a further practical method of refining the cathode deposit, or slimes, obtained in accordance with my process described above, to melt it into anodes for a second treatment by

my process, by the method described on the preceding page. This involves removing the admixed  $\text{AgCl}$  by one of the methods described on the preceding page, before melting. Part of the gold is deposited and part remains in the electrolyte.

When sufficient gold has deposited, the deposit with admixed  $\text{AgCl}$  and the electrolyte may be removed together, and the deposited gold brought into solution by the addition of nitric acid. For this method, the silver content of the cathode de-

posit may be kept low by high cathode current density and cooling, and by superimposed alternating current or rectified current, in which case, very little nitric acid is required. The solution is diluted and filtered free of silver chloride, and the gold is precipitated in the filtrate in pure form.

Another application of my process for refining the anodes made from the cathode slimes of the parting process involves dissolving the gold of the anode electrolytically and entirely prevent-

ing the formation of a deposit, by the familiar use of porous cups surrounding the cathode. The anode solution is diluted and filtered, separating the silver chloride, and fine gold precipitated chemically from the filtrate.

Superimposed alternating current upon direct current or rectified alternating current may be applied in the refining process as well as in parting, and the use of concentrated hydrochloric acid and the addition of soluble chloride is desir-

able but not essential in refining high gold content anodes.

To refine the spent electrolyte and washings, the spent baths are accumulated in a final precipitating tank. The silver, the platinum metals and traces of gold are precipitated together by hanging strips of copper or zinc in the tank.

However, if the anode is known to be high in platinum metals, the latter may be recovered directly from that particular lot of electrolyte.

The end tank precipitate can be removed and washed, and dissolved in aqua regia, and the various metals precipitated from the evaporated and diluted solution. Another method is to melt the precipitates into anodes and electrolytically

dissolve them in hydrochloric acid, using a porous cup to prevent cathode deposition.

The electrolyte I employ and which is set forth in this specification and in the claims as concentrated hydrochloric acid is concentrated hydrochloric acid of substantially commercial

strength and salted down with a small quantity of

nitric acid to mottled off of each of the parts of strength. As is well known in this art, commercial strength hydrochloric acid is available as

muriatic acid at  $18^\circ \text{Bé}$ ,  $20^\circ \text{Bé}$ , and  $22^\circ \text{Bé}$ .

Although I have described in detail several modifications and embodiments of my process, many variations may be made which come within the broader spirit and scope of my invention, and I do not intend to be limited except as set forth in the following claims.

I claim:

1. The method of parting a gold bullion anode of any purity which comprises electrolytically dissolving the gold in an electrolytic bath initially comprising commercial concentrated HCl free of gold salts.

2. The method of parting and refining a gold bullion anode of any purity which comprises electrolytically dissolving the gold in an electrolytic bath initially comprising commercial concentrated HCl free of gold salts and depositing the gold on the cathode as a non-adherent spongy mass and remolding the parted gold as an anode and repeating the process with the parted gold as an anode.

3. The method of parting a gold bullion anode of any purity containing silver in a bath initially comprising commercial concentrated HCl free of gold salts which comprises passing current of a density of the order of from 100 to 900 amperes per square foot between the cathode and anode to part the gold electrolytically from the anode and without the formation of passive  $\text{AgCl}$  on the anode.

4. The method of gold parting a gold bullion anode of any purity which comprises electrolytically dissolving the gold in an electrolytic bath initially comprising commercial concentrated HCl free of gold salts and superimposing a current to prevent polarization.

5. The method of gold parting and refining a gold bullion anode of any purity which comprises electrolytically dissolving the gold in a bath of commercial concentrated HCl, removing the gold from the HCl, and refining the gold by electrolytic deposition in a chlorauric acid bath.

6. The method of gold parting and refining a gold bullion anode of any purity which comprises electrolytically dissolving the gold in a bath of commercial concentrated HCl and electrolytically refining the gold in a concentrated HCl bath and depositing the gold.

7. The method of gold parting and refining a gold bullion anode of any purity which comprises electrolytically dissolving the gold in an electrolytic bath initially comprising commercial concentrated HCl free of gold salts and refining the gold chemically.

8. In an electrolytic system having an anode of any purity of gold bullion, an initial bath of commercially concentrated HCl free of gold salts and a cathode, the method of gold parting which comprises passing a current through the anode, electrolyte and cathode, removing the gold from the anode and depositing it on the cathode in the form of an impure loose spongy mass and refining the cathode deposit by dissolving the gold in aqua regia and chemically precipitating the gold from the aqua regia solution.

9. The method of gold parting which comprises passing an electric current from an anode of gold bullion of relatively low to high fineness through a bath of commercial concentrated hydrochloric acid, depositing metallic gold from the solution on the cathode in the form of a

75

50

50

55

60

65

70

75

75

75

loose spongy mass, and permitting the cathode deposit to drop to the bottom of the solution.

10. The method of gold parting which comprises passing an electric current from a gold anode of the order of .600 fine and containing silver of the order of 15% and copper of the order of 20% and other metals including metals of the platinum group through a bath of commercial concentrated hydrochloric acid, depositing metallic gold from the solution on the cathode in the form of a loose spongy mass, and permitting the cathode deposit to drop to the bottom of the solution.

11. The method of gold parting which comprises passing an electric current from an anode of impure gold through a bath of commercial concentrated hydrochloric acid containing a small amount of a chloride of a metal selected from the group of alkali and alkali earth metals, 20 depositing metallic gold from the solution on the cathode in the form of a loose spongy mass, and permitting the cathode deposit to drop to the bottom of the solution.

12. The method of gold parting which comprises passing an electric current of a density of the order of from 150 to 900 amperes per

square foot from an anode of impure gold containing silver through a bath of commercial concentrated hydrochloric acid, depositing metallic gold from the solution on the cathode in the form of a loose spongy mass, and permitting the cathode deposit to drop to the bottom of the solution.

13. The method of gold parting which comprises passing an electric current from a gold anode containing silver to a cathode through a bath of commercial concentrated hydrochloric acid at current densities of the order of from 150 to 900 amperes per square foot, forming silver chloride on the anode in the form of a loose spongy mass, depositing gold on the cathode in the form of a loose, spongy mass, and maintaining the concentration of hydrochloric acid sufficient to maintain the electrolytic action at a predetermined rate.

14. The method of gold parting which comprises passing an electric current at a current density of the order of 650 amperes per square foot from an impure gold bullion anode through an electrolytic bath initially comprising commercial concentrated hydrochloric acid to a cathode.

SAMUEL J. BLAUT.